

## UNITED STATES PATENT OFFICE

WILLIAM TROTTER, OF NEW YORK, AND ELTOFT WRAY WILKINSON, OF QUEENS VILLAGE, NEW YORK, ASSIGNEES TO MINERALS SEPARATION NORTH AMERICAN CORPORATION, OF NEW YORK, N. Y., A CORPORATION OF MARYLAND

## FLOTATION CONCENTRATION OF PHOSPHATE-BEARING MATERIAL

No. Drawing. Application filed January 24, 1928. Serial No. 249,197.

This invention relates to mineral concentration and is herein disclosed as applied to the concentration of phosphate mineral to produce a material rich in  $\text{Ca}_3\text{P}_2\text{O}_8$ , commercially known as bone phosphate of lime.

It has been known for a long time that some minerals other than metals and metalliferous sulphides are amenable to concentration by the froth-flootation process, but, in the case of phosphates at least, the consumption of agents, principally oil, was so great that the process was unavailable commercially because of the prohibitive cost of the agents in the necessary quantities, particularly when the process is carried out in reclaimed mine pit or washer waters.

According to the present invention these and other difficulties have been overcome. According to the procedures of the present invention the prepared phosphate rock is agitated in a pulp with a suitable soap and with an oily material which may be unsaponifiable or non-frothing, such as fuel oil. Frequently a proportion of one part soap to three parts oil has been found most useful. It is found that relatively coarse phosphate rock, for example, passing 14-mesh, can be floated with a relatively small consumption of such agents and without excessive agitation and aeration, yielding a high grade concentrate and yet with small loss of phosphate in the tailings.

The most satisfactory results have been obtained within the limits of cost of commercial operations when a substantial reduction of the ordinary proportion of primary slimes was effected before the prepared rock was submitted to the concentration process. Secondary slimes resulting from grinding the ore are often so much richer that the increased recovery from them may wholly or partly offset the increased cost of concentration arising from their presence due to increased consumption of soap and oil.

It is not necessary that the concentration

process be so conducted as to produce a froth-float. The process has been many times operated when a float concentrate was obtained in which the air bubbles were mainly concealed beneath a mat of coarse grains of phosphates as though the rock grains were in agglomerates too heavy to be supported by single bubbles or too stiff to conform to the shape of a single bubble. These grains behaved as if they had some tendency to cohere together and to adhere to the bubbles which had raised them. There were many bubbles in and below the mat which broke on passing through the mat.

With finer ground material a froth forms, carrying phosphates in or on its bubble films, but it does not appear to be necessary that much, or in some cases any, froth-flootation concentration be effected.

Most of the following tests represent work done in testing machines under exactly controlled and reproducible conditions, but parallel results have been obtained in operating an eighteen-inch ten-cell subaeration minerals separation machine, as will also appear.

Undersize phosphate rock from the No. 11 mill of International Agricultural Corporation at Mulberry, Florida, was subjected to a desliming operation until relatively free from slimes and then found to contain little material finer than 100-mesh. It was then screened to remove between five and six per cent of the material which was coarser than 14-mesh Tyler screen. 550 grams of the finer than 14-mesh wet material, carrying about 10 per cent. of water, was agitated in a minerals separation box-type subaeration testing machine with 500 cc. of tap water and there was added, in the order named, 10 cc. of a soap solution and 1.5 cc. of 39° Oklahoma fuel oil.

The soap solution was made by combining 88 grams single pressed red oil (oleic acid) 90

with 12.5 grams caustic soda, and adding enough water to make 2000 cc., so that 10 cc. of the solution contained one-half gram of soap.

5 The thick pulp with the soap and oil was agitated forty-five seconds and then water was added to fill the machine almost to overflowing and vigorous agitation started and air admitted. The float soon rose and overflowed, with some assistance from a paddle for one minute and forty-five seconds. The concentrate as it lay on the collecting launder was composed of clean grains not unlike wet yellow sea sand. It had practically no trace 10 of the froth films which were obtained with and persisted with the concentrate obtained in treating finer material. The results are shown in terms of bone phosphate of lime in the following table:

20

|       | Wts. | Assays | Recoveries |
|-------|------|--------|------------|
| Heads | 100. | 44.6   | 100.       |
| Conc. | 51.4 | 73.9   | 85.        |
| Mid   | 11.8 | 46.    | 12.        |
| Tails | 36.8 | 3.3    | 2.7        |

30 In another test the same material subjected to the same desliming operation, was used. 550 grams were mixed with 500 cc. water, to which was added, in the order named, 10 cc. 35 of a fish-oil soapy emulsion and 3 cc. of the same fuel oil. The fish-oil emulsion was made by warming 25 grams of a dark pressed fish-oil, several years old, with 100 cc. of water and 13 cc. of a 10 per cent. solution of caustic soda, so that 10 cc. of the final solution contained 1.9 grams of oil and 0.1 grams of caustic soda.

40 The thick pulp with the emulsion and oil was slowly agitated for 30 seconds. Then water was added to fill the machine almost to overflowing and vigorous agitation started. The float soon rose and overflowed. A froth 45 of the type usual in froth-flotation appeared only at the end of the frothing period, when the greater part of the phosphate mineral had been removed. The concentrate was removed for two and one-half minutes, and 50 separated by retreatment into a finished concentrate and a middling. The results are shown in the following table:

|       | Wts.   | Assays | Recoveries |
|-------|--------|--------|------------|
| Heads | 100.00 | 47.1   | 83.0       |
| Conc. | 49.5   | 79.0   | 5.0        |
| Mid   | 4.8    | 49.4   | 11.9       |
| Tails | 45.7   | 12.2   |            |

60 Another lot of the same material subjected to the same desliming operation, but ground to pass 48-mesh and 61 per cent. passing 150-mesh, and carrying all the slime formed in grinding, was concentrated as follows:

500 grams of the dry material was slowly mixed with 500 cc. of water and there was added 25 cc. of a 5 per cent. solution of pure sodium oleate and 5 cc. of fuel oil. After one minute enough water was added to fill the machine and vigorous agitation started. The float was collected during 1 1/4 minutes. The first float was a heavy froth concentrate in which bubble films survived when separated from the pulp. The concentrate was retreated to give a finished concentrate, and a middling. The results are shown in the following table:

|       | Wt.  | Assays | Recoveries | 80 |
|-------|------|--------|------------|----|
| Heads | 100. | 44.6   | 100.       |    |
| Conc. | 51.4 | 73.9   | 85.        |    |
| Mid   | 11.8 | 46.    | 12.        |    |
| Tails | 36.8 | 3.3    | 2.7        |    |

85 A pulp of phosphate pebble screenings of the Mulberry Florida, mine passing approximately 20-mesh was subjected to a desliming operation until relatively free from slimes and was concentrated by feeding at the rate of about nine tons of solids per hour through a ten-cell Wilkinson and Littleford subaeration impeller flotation machine, with the addition at the first-cell of sodium oleate 3.9 pounds and fuel oil 12.4 pounds, both per ton of solids, together with a very small quantity of pine oil. Only enough water was used in the first two cells to make an easily mixed pulp, estimated to contain 60% solids. 90 Enough water was added at the third cell to make a pulp estimated to contain 17% of solids, and the float was removed in this and later cells.

95 The heads contained 39.4% bone phosphate of lime, the concentrates 71% and the tailings 10.2% making a commercial yield, with a recovery of 86.5%.

100 In one continuous mill run about 65 to 70 tons of similar material passing about 28-mesh was subjected to a desliming operation until it contained a very small proportion of slimes. It was agitated in a thick pulp with 4.9 pounds of oleic acid soap and 8.06 pounds 105 of Mexican fuel oil, both per ton of solids. The feed contained 29.22% bone phosphate of lime. The pulp was thinned, further agitated, and a concentrate was obtained containing 72.8% of bone phosphate of lime, and the tailings contained 5.16% of bone phosphate of lime, representing a recovery of 89% and a ratio of concentration of 2.8 to 1.

110 The product was commercially marketable in that form, but tests have shown that such concentrates can often be profitably recleaned. For example, material of the same general character was ground to pass 20-mesh, 28-mesh, 48-mesh, and 100-mesh. Each size was 115

concentrated separately yielding rough concentrates and rough tailings, and final concentrates, middlings and final tailings, having the contents of bone phosphate of lime shown in the following table:

| 10        | Assays—per cent |       |           |      |       |    |
|-----------|-----------------|-------|-----------|------|-------|----|
|           | No retreatment  |       | Retreated |      |       | 15 |
|           | Conc.           | Tail. | Conc.     | Mid. | Tail. |    |
| —20 mesh  | 70.8            | 6.0   | 76.8      | 36.8 | 6.6   |    |
| —28 mesh  | 67.4            | 3.8   | 74.8      | 34.4 | 5.4   |    |
| —48 mesh  | 67.6            | 8.2   | 76.4      | 49.4 | 8.6   |    |
| —100 mesh | 65.6            | 12.8  | 74.4      | 60.8 | 9.8   |    |

The agents used were 6 pounds of sodium oleate and 18 pounds of Oklahoma fuel oil, both per ton of solids, and, except for the addition of a further 2 pounds of sodium oleate, per ton of solids in treating the 100-mesh material, no agents were added for retreating the materials.

Other tests indicated that much less soap and oil would have yielded an equally good result with the coarser materials.

Addition of the soap and oil to a thick pulp containing as much as 60% solids and disseminating by agitation thereof and thereafter thinning to yield a float frequently proves economical, partly because less of the soap is consumed in softening the water, partly because less oil seems to be needed when the smaller quantity of soap is used, and partly because less equipment is needed, though useful results may be obtained by agitating in the freely flowing pulp which was to yield the float. Satisfactory dissemination was obtained in a pulp so thick that it would barely flow down a 30° grade, until later diluted for flotation.

In one test run the crude phosphate ore passing 20-mesh was subjected to a desliming operation until free from primary slimes. The subaeration machine was started slowly with 400 cc. of water, and then was added 500 grams of the crude phosphate ore, so that the pulp contained 55 5/9% of solids. Cotton-seed oil soap was added at the rate of 2.6 pounds followed by Oklahoma fuel oil at the rate of 6 pounds, and pine oil at the rate of 0.12 pounds, all per ton of solids. The machine was then brought up to full speed for 15 seconds, then slowed and water added to make a freely flowing pulp containing 17% solids. The speed was then increased and air admitted so that a float rose, and this float was removed for three minutes. The tailings were removed, the concentrates put back in the machine with 0.12 pounds additional pine oil per ton of original ore, water added to nearly fill the machine, agitation resumed, air admitted and the finished concentrates

removed for one and one-half minutes. The results are shown in the following table:

| Product | Wt.—per cent | Bone phosphate of lime—per cent | Recoveries of same—per cent | 70 |
|---------|--------------|---------------------------------|-----------------------------|----|
| Heads   | 100.         | 36.30                           |                             |    |
| Cone    | 35.6         | 72.77                           | 71.2                        |    |
| Midds.  | 7.6          | 47.80                           | 9.7                         |    |
| Tails   | 56.8         | 12.22                           | 19.1                        |    |

75

Other phosphate ores require some modifications in treatment. It is found that very small amounts of silicate of soda may be sometimes advantageously added to the pulp, especially after the addition of the other agents. Other bubble-forming agents than pure soap have been found helpful in the presence of soap, such as cresol or the pine oil mentioned above or the sulphonated castor oil known as Turkey red oil. Many other soaps, have been satisfactorily used, such as cotton-seed oil soap, laundry soaps, borax soaps and rosin-containing soaps, but one pure cocoanut oil soap gave no useful result. Saponified rosin in one test proved useless. The exact nature of the soap makes some difference in the results, and freshly prepared soaps sometimes proved best. Moreover commercial soaps sometimes proved more satisfactory than the chemically pure soaps.

Microscopic examination of the prepared phosphate rock showed that its gangue was mainly transparent silica and that the binding of silica to phosphate was well destroyed in the 14-mesh material.

Having thus described certain embodiments of the invention, what is claimed is:

1. The process of concentrating phosphate-bearing material which consists in subjecting such material to a desliming operation, then agitating and aerating a pulp of the material with oil and with a compound adapted to control selective oiling of the phosphate so as when cooperating with such oil to yield a floating concentrate, and separating the float.

2. The process of concentrating phosphate-bearing material which consists in agitating and aerating a pulp of the material with soap and a non-frothing oil so as to yield a floating concentrate, and separating the float.

3. The process of concentrating phosphate-bearing material which consists in subjecting such material to a desliming operation, then agitating and aerating a pulp of the material with soap and oil so as to yield a floating concentrate, and separating the float.

4. The process of concentrating phosphate-bearing material which consists in agitating and aerating a pulp of the material with soap and petroleum oil so as to yield a floating concentrate, and separating the float.

5. The process of concentrating phosphate-bearing material which consists in subjecting such material to a desliming operation,

95

100

105

110

115

120

125

- then agitating and aerating a pulp of the material with soap and oil in the proportion of about one to three, the soap being used in about that proportion to the area of the surfaces of the particles of phosphate material which two pounds bears to the surfaces of twenty-mesh material, the agitation and aeration being so conducted as to yield a floating concentrate, and separating the float.
6. The process of concentrating phosphate-bearing material which consists in subjecting such material to a desliming operation so that it is practically free from sizes coarser than 14-mesh, then agitating and aerating a pulp of the material with soap and fuel oil so as to yield a floating concentrate, and separating the float.
7. The process of concentrating phosphate-bearing material which consists in subjecting such material to a desliming operation to yield floatable sizes containing a minimum of slimes then agitating and aerating a pulp of the material with soap and oil so as to yield a floating concentrate, and separating the float.
8. The process of concentrating phosphate-bearing material which consists in agitating with soap and petroleum oil a pulp of the material which is too thick to flow freely so that the phosphate is selectively oiled, diluting the pulp with water to make a freely-flowing pulp, agitating and aerating the diluted pulp to produce a floating concentrate, and separating the float.
9. The process of concentrating phosphate-bearing material which consists in subjecting such material to a desliming operation, then agitating with soap and petroleum oil, in the proportion of about one to three, a pulp of the material which is too thick to flow freely, the soap being used in about that proportion to the area of the surfaces of the particles of phosphate material which two pounds bears to the surfaces of twenty-mesh material, diluting the pulp with water to make a freely-flowing pulp, agitating and aerating the diluted pulp to produce a floating concentrate, and separating the concentrate.
10. The process of concentrating phosphate-bearing material containing gangue, which consists in subjecting such material to a desliming operation, then agitating and aerating a pulp of the material with oil and with a compound adapted to control selective oiling of the phosphate so as to effect the lifting in the pulp of phosphate-bearing particles above gangue particles by attached air bubbles, and collecting phosphate-bearing particles relatively free from gangue particles.
11. The process of concentrating phosphate-bearing material containing gangue, which consists in agitating and aerating a pulp of the material with soap and a non-frothing oil so as to effect the lifting in the pulp of phosphate-bearing particles above gangue particles by attached air bubbles, and collecting phosphate-bearing particles relatively free from gangue particles.
12. The process of concentrating phosphate-bearing material containing gangue, which consists in agitating with soap and petroleum oil a pulp of the material which is too thick to flow freely so that the phosphate is selectively oiled, diluting the pulp with water to make a freely-flowing pulp, agitating and aerating the diluted pulp so as to effect the lifting in the pulp of phosphate-bearing particles above gangue particles, and collecting phosphate-bearing particles relatively free from gangue particles.
- In testimony whereof, we have affixed our signatures to this specification.
- WILLIAM TROTTER.  
ELTOFT WRAY WILKINSON.

85

90

95

100

105

110

115

120

125

130